

# UNITED STATES PATENT OFFICE.

ROBERT J. TILFORD AND HENRY M. REDEMAN, OF LOUISVILLE, KENTUCKY,  
ASSIGNORS TO THE REDEMAN-TILFORD STEEL COMPANY, OF SAME  
PLACE.

## MANUFACTURE OF STEEL.

SPECIFICATION forming part of Letters Patent No. 397,476, dated February 5, 1889.

Application filed July 25, 1888. Serial No. 281,018. (Specimens.)

*To all whom it may concern:*

Be it known that we, ROBERT J. TILFORD and HENRY M. REDEMAN, citizens of the United States, residing at Louisville, Kentucky, have invented new and useful Improvements in the Process of Hardening Steel, of which the following is a specification.

Our invention relates to certain new and useful improvements in the treatment of crude or low-grade steel to produce a refined or high-grade steel.

The most successful method of producing low-grade steel is that known as the "Bessemer" process, described in his patent of 1855; but this product, as is well known, is suitable chiefly for railways, axles, and like uses, and is totally unsuited for structures, machinery, and tool purposes unless repuddled, hammered, and rolled, for the reason that in its normal state it is too soft, and when hardened it becomes too hard and brittle for the purposes stated. It was the recognition of these inherent defects in the Bessemer and low and medium grade steel which led us to the investigation of the subject which has developed our present invention, the object of which is the production at slight cost and a minimum degree of labor of a higher grade and more refined steel by treating the Bessemer and other low-grade steel in such manner as to produce a molecular change from a coarse grain to a fine grain and silky fracture, to increase the tensile strength, elasticity, toughness, and ductility, and to greatly increase the carbon. We have found from experience that uniform results in all instances flow from the treatment of metals having like properties.

With these ends in view our invention consists in heating low-grade steel to a degree of heat represented by white heat, and then subjecting the metal so heated to a previously prepared liquid bath of such character that the contact of the heated metal and liquid-bath will generate hydrocarbon gases, which will be absorbed or taken up by the metal, and allowing the metal to remain in the bath until it has become substantially cool, in contradistinction to what is known as the cementation or dry process, as will be hereinafter more fully set forth.

As an illustration of one of the baths employed in the practice of our invention, we would state that we employ glycerine and water in the proportion of three (3) ounces of glycerine to one-half ( $\frac{1}{2}$ ) gallon of water, and allow the heated metal to remain submerged until the change is effected, which should be until the metal is substantially cool, or until such reduction in heat in the metal is made that it will no longer take up the gases generated by contact with the bath. We have also found that by adding to the bath of glycerine and water spirits of niter, aqua-ammonia, chloride of ammonium, sulphate of zinc, sulphate of alumina, and ammonia the results and effects obtained by a bath of glycerine and water alone are improved, although good results are obtained by the latter.

In practicing our invention by the last-named bath we employ the several chemical bodies in about the following proportions, to wit: spirits of niter, one and a half ( $1\frac{1}{2}$ ) ounce; aqua-ammonia, one and a half ( $1\frac{1}{2}$ ) ounce; chloride of ammonium, two (2) ounces; sulphate of zinc, one and a half ( $1\frac{1}{2}$ ) ounce; sulphate of alumina and ammonia, one and a half ( $1\frac{1}{2}$ ) ounce; glycerine, three (3) ounces; water, one-half ( $\frac{1}{2}$ ) gallon.

We desire to state herein, however, that we lay no specific claim to either of the baths described above by which we practice our invention, as the one first described forms the subject-matter of a divisional application of this case filed on 13th day of November, 1888, Serial No. 290,737, while the second bath described forms the subject-matter of a second divisional application filed on the same day and bearing Serial No. 290,738, to which divisional applications reference is made for a more full and complete description of the manner of carrying out the generic idea which the present application is intended to cover.

As further explanatory, however, of the advantages gained by the present invention, we would state that by the practice of our process (which should be understood as being distinguished from processes for tempering steel in oil) the nature, the physical construction, and the molecular construction of the metal are completely changed, whereas the

tempering of steel in oil, as practiced by some processes, simply tempers the steel more slowly than is done by tempering in water and other properties, leaving the metal less hard, but somewhat tougher than water-tempered material. The changes caused by the oil-tempering process are merely temporary, and do not change the physical or granular construction of the metal, and such changes as are caused thereby can be readily neutralized by reheating and allowing the metal to cool. The changes caused by treatment by our process are permanent, and cannot be removed by any known treatment or process without entirely destroying the steel properties of the metal by burning.

We have of course been unable to analyze the gases resulting from the contact of the hot-metal body with the bath, but are led to believe that they constitute a hydrocarbon gas which has a strong affinity for the metal, and that the latter, being in a heated state, is in such a physical condition as to readily take up or absorb such gas; but as to the fact that the metal is highly improved we have no doubt whatever, as has been demonstrated by all the well-known scientific and mechanical tests.

It will be understood, of course, that when the treatment is applied adjacent to the furnaces where the low-grade steel is manufactured the ingots may be treated without re-heating, and thus the expense of such re-heating is avoided. After the metal has been subjected to the treatment it is allowed to cool in the ordinary manner, and it may afterward be subjected to any ordinary hardening or tempering process, and the temper may, if necessary, be drawn and again restored without at all affecting the other properties acquired from the bath.

We are of course aware that the quality of Bessemer and other low and medium grade steel may be improved by what is known as the "dry" or "cementation" process, which requires a large expenditure of skilled labor

and great length of time, and that, too, without always securing uniform and satisfactory results.

We desire it to be distinctly understood that we lay no claim to the broad idea of increasing the quality of steel by subsequent treatment, as that has been heretofore done, especially by what is known as the "cementation process," which may be termed a "dry process," our invention differing from such process in the particular that it requires a period of time amounting to a small percentage of the time required in the cementation or dry process, and is in contradistinction to such process essentially a liquid or wet process, the former requiring many days, while the latter involves only a few minutes.

By our invention we greatly increase the tensile strength and elasticity, and yet do not destroy the per cent. of reduction or ductility, while with ordinary tempering the tensile strength and elasticity are greatly increased, but the per cent. of reduction and ductility is very much impaired.

Having thus described our invention, what we claim as new, and desire to secure by Letters Patent, is—

The process of converting low-grade steel into refined or high-grade steel, which consists in first heating the metal to be treated to a degree of heat represented by white heat, and then subjecting the metal so heated to a previously-prepared liquid bath, which by contact with the heated metal gives out hydrocarbon gases which are taken up by the heated metal, and allowing the metal to remain in such bath till practically cooled, substantially as hereinbefore set forth.

In testimony whereof we have hereunto set our hands in the presence of two subscribing witnesses.

ROBERT J. TILFORD.  
HENRY M. REDEMAN.

Witnesses:

W.M. C. MCINTIRE,  
CURTIS LAMMOND.